

Sept. 8, 1931.

H. F. WINKELMANN

1,822,636

INSULATING MATERIAL

Filed March 5, 1930



*Henry F. Winkelmann.*

Inventor

By *C. Snow & Co.*  
Attorneys.

## UNITED STATES PATENT OFFICE

HENRY F. WINKELMANN, OF NEBRASKA CITY, NEBRASKA

## INSULATING MATERIAL

Application filed March 5, 1930. Serial No. 433,396.

This invention relates to a material for use as a weatherproof covering, a heat and cold insulator and a sound deadener and it is more especially an improvement upon the preparation covered by Patent 1,743,744 issued to me on January 14, 1930. It is particularly useful as a roof covering, a wall insulator and as a sound proofing material for floors.

19 One of the objects is to provide a material which is extremely light, can be made at a low cost, and can be molded into slabs of desired proportions ready to be placed in position for use.

20 With the foregoing and other objects in view which will appear as the description proceeds, the invention resides in certain novel features hereinafter more fully described and pointed out in the claims it being understood that changes may be made without departing from the spirit of the invention as claimed.

In the accompanying drawing a portion of a slab embodying the present improvements has been shown.

The composition used in making the insulating material consists of the following ingredients substantially in the proportions stated, namely,

|               | Per cent<br>by volume |
|---------------|-----------------------|
| Asphalt       | 30                    |
| Paraffine oil | 5                     |
| Flax fibre    | 15                    |

35 To the foregoing ingredients there is added 50% of phlogopite which has been heated to approximately 2500° F. Phlogopite thus treated is extremely light and is formed of flakes which adhere in small lumps easily broken. Thus when the several ingredients are thoroughly mixed while heated the phlogopite in small pieces is scattered throughout the body of the mixture and gives it bulk and lightness.

40 The material while warm is adapted to be poured out to form a layer of any desired thickness. This layer can be provided with a base of black asphalt paper and with a top covering of the same material. After the 45 formed layer has cooled and reached its max-

imum degree of hardness, it can be cut into slabs ready for use. If preferred the material when used for roofing purposes, etc., can be moulded in a single slab at the place where it is to be left.

55 In the drawing which illustrates a portion of a slab having the present improvements, the phlogopite has been shown at 1, the balance of the mixture at 2, and the layers of paper at 3.

60 The advantage resulting from the use of phlogopite is that the composition is rendered fire-proof, sound-proof, and moisture-proof. This results in the formation of small air spaces in the material.

65 The asphalt when mixed with the paraffin oil produces a rubber-like pasty substance which can be formed easily into a slab. The flax fiber constitutes an efficient reinforcement while the paper serves to hold a slab in proper shape during the process of manufacture of a slab.

70 While this composition has been described as useful as a roof covering, a wall insulator, and a sound-proof material for floors, it is 75 peculiarly suited for use in basements and all under-ground work where it is desired to employ a material which will not rot.

What is claimed is:

1. A material of the class described including layers of asphalt paper spaced by an adhering mixture consisting of asphalt, vegetable fibre, paraffine oil, and flaked phlogopite.

80 2. A material of the class described comprising layers of asphalt paper spaced by an adhering mixture including the following ingredients substantially in the proportions stated, namely, asphalt 30%, paraffine oil 5%, flax fibre 15%, and flaked phlogopite 50%.

85 In testimony that I claim the foregoing as my own, I have hereto affixed my signature.

HENRY F. WINKELMANN.

95